

## UNITED STATES PATENT OFFICE

2,120,562

REFRACTORY MATERIAL AND PROCESS OF  
MAKING SAMEClemens A. Laise, Tenafly, N. J., assignor to  
Eisler Electric Corporation, Union City, N. J.,  
a corporation of DelawareNo Drawing. Application October 11, 1934,  
Serial No. 747,891

16 Claims. (Cl. 75—137)

The present invention relates to hard metal compositions, to methods of working such hard metal compositions, and to processes for producing compositions of this description that are 5 adapted for working into shapes suitable for various commercial uses.

Such shapes may take many forms. Among others may be specifically mentioned the form of borers for oil well drilling, sand blast nozzles, 10 tips for cutting tools, nibs for wire-drawing dies, high resistance insulators for radio circuits and parts and contacts for all types of mechanical and electrical apparatus subject to extreme wear and tear.

15 It is an advantage also that the material of the invention is practically non-corrosive and may consequently be employed for many uses where materials of the prior art are damaged by corrosion, tarnish or rust, or by electrolytic 20 action.

I am aware that there are a number of processes for producing hard metal compositions, some of which include in the composition some of the basic elements mentioned in the present invention. In the past, however, it has been customary, in making such hard metal compositions, first to provide a finely divided carbide of a refractory metal; then to press and sinter such carbide into a form or shape. The resulting 25 form or shape was naturally of a rather brittle and porous character but extremely hard. Therefore, in order to add toughness to the article so produced, it was necessary to impregnate it with a cementing metal. This cementing metal 30 was introduced into the pressed and sintered carbide form or shape, generally either by mixing the cementing metal in finely divided form with the carbide before pressing and sintering, or else first pressing and sintering the carbide, and then 35 dipping the shape or form into a molten bath of cementing metal.

In contradistinction to these methods and other similar processes of the prior art, the present invention comprehends the mixing, before 45 carbidization, of a refractory metal or metals with a base metal or metals, both in very finely divided form. I have discovered that if such a mixture is then heated to a temperature just below that of the sintering temperature of the lowest melting point metal in the mixture, there is a relatively rapid combination or alloying of the metal contained in the mixture. This alloy is then very readily carbidized at surprisingly low temperatures as hereinafter set forth, and subsequently treated in such a manner as to form a

material suitable to be used in the extruding steps hereinafter set forth. The carbidized alloy may be treated by breaking it up into an abrasive metallic powder suitable for directly forming hard metal members without the formation of 5 the extrusion material or the practice of the extruding steps.

Under the processes of the prior art, it seemed to be necessary to produce shapes such as above described, which might take the forms of polygonal, fluted or cylindrical rods or of tubes, by machining the same or by pressing or molding various types of hard metal compositions into the forms desired, or by first putting the material into cylindrical form and subsequently shaping 10 the same. Due, however, to the extreme hardness of such materials, it was very difficult to machine or cut shapes so made, once they were formed. This was particularly true after the material had been subjected to the heat treatment 15 which usually accompanied the application of pressure.

It is an object of the present invention to provide a material and a method of producing the same that will permit of easily forming and 20 cutting into the desired shape and size, and which material and method greatly increase the variety of shapes into which hard metal compositions may be processed.

The invention comprehends a material especially adapted for the purposes above mentioned, the steps of preparing this material, the steps of shaping the material so prepared into the desired forms and the steps of hardening the shapes so formed into a usable, commercial condition. The 25 achievement of these ends is among the objects 30 of the invention.

More specifically, the invention comprehends an extrusion material, process and product. The extrusion material may be generally described as 35 a refractory metal composition in plastic state; the process includes the mixing and alloying, and the carbidizing of a refractory and a base metal and the extrusion, drying, baking, cutting and hardening of this material; and the product may 40 be represented by shaped members resulting from the application of the process to the said material.

To accomplish these ends a mixture is prepared comprising very finely divided refractory 45 metals and base metals. The refractory metals should for best results consist of a mixture of any two or more of the following: Tungsten, tantalum, titanium, zirconium, chromium, thorium or rhenium, etc. In fact, any carbide form- 50

ing metals having a melting point above 1500° C. may be used. These or some of these metals of such refractory nature are then in proper cases mixed with one or more of such other metals 5 having a melting point of 900° C. or above, as iron, manganese, nickel, cobalt, silver, copper, etc., also in very finely divided state.

I have discovered that it is possible to produce a remarkable change by intimately mixing and 10 milling finely divided refractory metal powders such as tungsten and molybdenum, etc., with base metal powders such as iron, nickel or cobalt, without heating the mixture to the lowest melting point of any of its constituents. To produce 15 this result constitutes the first step in the procedure. The mixture of powders above mentioned is heated in a hydrogen atmosphere in a suitable gas or electric furnace at a temperature of 700° C. to 900° C. and preferably at temperatures just under the melting points of the 20 base metal constituents for a period of several hours. Under this treatment a light sintering takes place permitting subsequent crushing and sieving; but more than this, an apparent absorption 25 of some of the elements into others takes place, thus forming substantially homogeneous particles having the characteristics of alloys. For instance, copper and nickel will readily intimately intermix in this manner so that a red 30 50% mixture, after heat treating will result in a white or silvery powder no longer resembling the original mixture and having characteristics of an alloy. Similarly, tungsten or cobalt, or tungsten and nickel, may be intimately intermixed and alloyed in the powder form. This preliminary intimate intermixing, alloying and sintering stage is, therefore, an important step in my 35 process, as it greatly facilitates the preparation of the material with which the subsequent extrusion step is carried out.

The next step is the formation of carbides from these intimate mixtures or alloys of metal powders. The sintered alloy metal powders consisting of refractory metals intimately admixed with base metals, preferably of the iron group, are 40 carbidized by uniformly mixing carbon or carbon and boron, also in fine division, with them in order to form a combination of such alloys with nonmetallic elements such as carbon and boron and to facilitate the formation of carbides or 45 borides or both. Such sintered powders can be carbidized at temperatures much lower than merely the powdered mixtures of the same composition. Thus, I find to carbidize tungsten powder in itself requires a temperature of 200° C. 50 to 400° C. higher than when I carbidize a sintered tungsten-nickel alloy powder containing 70% tungsten and 10% nickel. The amount of carbon should be calculated to provide an amount sufficient to cause the carbide-forming metals to 55 absorb the normal atomic ratio of carbon to metal to give the desired carbide molecule. The carbon may, however, be added during the heat treatment which follows by heating in an atmosphere of carbonaceous gas. For facility of explanation I shall refer hereinafter to "carbides" with the understanding that what is said of carbides applies equally to borides or carbides and borides.

In order to effect carbidization, the alloyed 60 metal powders and carbon are subjected to a heat treatment at a temperature elevated to or almost to the sintering temperature of the mixture and below the melting point thereof, say 75 1200° C. to 1400° C., for a period of from two to

six hours. This operation is carried out in a hydrogen, carbonaceous or reducing atmosphere. The result is either a still finely divided product consisting of carbides, or borides, or, in a case where both carbon and boron are added, of both carbides and borides of the alloyed metals in the mix. Where the temperature of the heat treatment is sufficiently high, the powdered metal carbides resulting are in the form of wholly or partially sintered masses or at any rate usually 10 contain lumps throughout the mass. In order to facilitate the production of the extrusion material hereinafter referred to, it is necessary to crush or grind this material and ball mill it to bring it back to a very fine state of subdivision, 15 the particles being capable of passing through a sieve of the order of 350 mesh. The sintered carbidized alloy, however, may be crushed or ground to form an abrasive metallic powder which may be used to produce hard metal members by other methods than by the extrusion process herein described.

From this carbidized or boridized fine alloy powder thus prepared, the extrusion material of the present invention is formed and its formation constitutes the next step.

The nature of this extrusion material is determined by the requirements necessitated by the conditions of the extruding procedure which will be described hereafter and, to a certain extent, 30 by atmospheric conditions.

The formation of the extrusion material is best begun by forming a suitable paste which may act as a binder for the finely divided alloy carbide. This paste may consist of starch, water 35 and ammonia, in the proportions of 150 grams of starch to 825 cc. of water to 75 cc. of ammonia. In place of the foregoing paste, organic binding materials, such as a caramel solution, gum arabic, or a casein solution, or mineral binders, such as 40 silicates or mineral colloids may be used. In any case the quantity of paste must be such as to render the mixture sufficiently viscous so that the extruded mass will hold together into a compact body having a smooth surface and free from 45 pores or voids. If the mixture of alloy carbides and paste contains an improper quantity of paste, the extruded pieces may show minute cracks on the surface. In this case the pieces must be broken up and remixed with the proper proportion 50 of paste until the proper consistency for yielding dense, smooth-surfaced products is attained.

The paste may be mixed by the use of any standard heavy duty mixing equipment and 55 should be carried out until a thorough intermixture of ingredients into a plastic mass is obtained. A suitable consistency has been obtained by mixing refractory carbide powders and a starch paste compounded as above described 60 in the proportion of about 160 grams starch binder to 1 kilogram of carbide. The consistency of the composition may vary slightly under varying atmospheric conditions, but a mixture of the correct consistency may be produced under any 65 given set of conditions by a suitable variation in the amount of binder material. In some cases the paste may be rolled between or under suitable rolls of standard rolling mills so as to render the powders exceedingly fine and the paste hard 70 and plastic so that it must be extruded with the aid of hydraulic pressure.

Extrusion is accomplished by placing this plastic mass obtained as above outlined in an extruding apparatus and forcing the composition 75

through an orifice of suitable shape under hydraulic or other pressure, in excess of one hundred pounds per square inch. Channels or plates of plaster of Paris or glass may be provided adjacent to the extrusion nozzles in order to carry the extruded forms as they are produced. The extrusion equipment should be kept clean and free from imperfections in order to avoid the formation of scores and faults in the extruded products.

10 The next step in the formation of the shaped members of hard metal composition characterizing the final product comprises drying the extruded shapes preferably at room temperature and under a slightly humid atmosphere for a period of two or three days or longer.

15 They are then cut to the desired lengths and baked in a sintering furnace in order to carbonize the binding material with which the plastic mass was formed. A temperature of 500° to 20 700° C. for about one hour or less has been found sufficient to carbonize the binding and plasticizing material. The extruded members may be packed in carbon boats surrounded by lamp black during this baking treatment, during which a 25 reducing atmosphere may be maintained to advantage.

25 The final step comprises a further heat treatment for bonding together the particles into a uniform, homogeneous, strong, compact, wear-resisting body. The carbonized members produced by the baking treatment are again packed in carbon boats, surrounded by lamp black, and then heated in an electric furnace at a temperature of 1400° to 1500° C. This operation is carried out from 5 to 30 minutes, depending upon the shape and size of the extruded members. Preferably a carbonaceous or hydrogenous atmosphere is maintained in the furnace during this compacting and hardening step.

35 40 During the cohesion and adhesion of the particles together under the conditions of the final compacting and hardening step, a considerable shrinkage of the original extruded product takes place, ranging from 10 to 30%. Shrinkage in length is generally about 22% and in diameter about 27%, although small pieces manifest considerably less shrinkage. Uniformity in shrinkage is facilitated by maintaining as smooth a surface as possible on the extruded members.

45 50 An example of the composition of my novel product is as follows:

|                                     | Per cent     |
|-------------------------------------|--------------|
| Refractory metal (such as tungsten) | 92.5 to 57.5 |
| Iron                                | .25 to 5     |
| Chromium and thorium                | .25 to 2.5   |
| Carbon and boron                    | 5.0 to 10.0  |
| Cobalt and nickel                   | 2.0 to 25.0  |

55 60 The composition of the starting material is adjusted with reference to the additions and losses taking place during the processing, and also with the purpose in mind for which the end product is to be used. If the final composition is to be exceedingly hard, the metallic constituents should be held to a refractory metal content above 90% and a base metal content below 10%. If, on the other hand, the composition is to be extremely tough, the base metal content is increased above 65 70 10% or 12% and the refractory metal content proportionately reduced.

75 A more specific composition for a superior wear-resisting material comprises in its final stage a compact homogeneous body composed of a carbidized alloy of tungsten, chromium, iron,

and cobalt. This may be still further hardened through the incorporation of  $\frac{3}{4}$  to 1% of thorium. The final body consists of approximately the following composition:

|                        | Per cent | 5  |
|------------------------|----------|----|
| Tungsten               | 78.5     |    |
| Iron                   | 0.5      |    |
| Chromium and thorium   | 1.0      |    |
| Carbon and boron       | 6.5      |    |
| Cobalt (and/or nickel) | 13.5     | 10 |

15 In cases where a combined carbidizing and boridizing effect is desired, I may add powders of boron suboxide or boron nitride or other suitable boron compounds to the original mixture before the heat treating and alloying step, or immediately prior to carbidizing. In this case the total carbon and boron in the composition should not exceed about 15%.

20 By the above extrusion process I produce extruded metallic bodies which are not only exceedingly hard but also exceedingly tough, the hardness exceeding 85 on the "A" Rockwell hardness scale, and the tensile strength exceeding 200,000 lbs. per square inch. At the same time 25 my composition is exceedingly compact and dense. The harder and more compact the paste is before extrusion the more dense and pore-free is my composition. In fact, before extruding, my paste may even be rolled between metallic rolls so as 30 to make the powders exceedingly fine and the paste exceedingly hard so that it must be extruded on a hydraulic or power press.

35 Having thus described my invention, what I claim is:

1. An extrusion material comprising in a finely divided state a carbidized alloy of two or more refractory metals of the group consisting of tungsten, tantalum, titanium, zirconium, chromium, thorium and rhenium, and a metal of the group consisting of iron, nickel, cobalt, manganese, silver and copper, in intimate admixture with a paste containing carbonizable material, said paste being present in said mixture in quantity sufficient to impart to the whole the capability of being extruded through an orifice in the 45 form of a dense, coherent body.

2. An extrusion material comprising a carbidized alloy of tungsten and another refractory metal with a base metal, said metals being in powdered form and in intimate admixture with a paste consisting of carbonizable binding material and water, said paste being present in quantity sufficient to impart to the whole the capability of being extruded through an orifice in the 55 form of a dense, smooth, coherent body.

3. An extrusion material comprising a finely divided carbidized alloy of tungsten and another refractory metal with a base metal, said finely divided carbidized alloy being in intimate admixture with a paste containing carbonizable 60 binding material and water.

4. The method of making hard metal members comprising intimately intermixing finely divided powders of one or more refractory metals of the group consisting of tungsten, tantalum, titanium, zirconium, chromium, thorium and rhenium, with finely divided powders of one or more base metals of the group consisting of iron, manganese, nickel, cobalt, silver and copper, sintering and alloying said mixture and then carbidizing the same, finely dividing the carbidized product, thoroughly mixing therewith a paste of carbonizable material and thereby forming said carbidized material into a plastic mass, extruding said mass into a shape of the desired form, dry- 70 75

- ing the same and cutting the dried shapes approximately to size, carbonizing said shapes and finally firmly cohering the carbonized product by baking at a temperature just below the melting point of the base metals.
5. The method of making hard metal members comprising intimately intermixing finely divided powders of one or more refractory metals of the group consisting of tungsten, tantalum, titanium, 10 zirconium, chromium, thorium and rhenium, with finely divided powders of one or more base metals of the group consisting of iron, manganese, nickel, cobalt, silver and copper, sintering and alloying said mixture and then carbidizing the same, finely 15 dividing the carbidized product and forming a plastic mass thereof, extruding said mass into a shape of the desired form, drying the same and cutting the dried shapes approximately to size, carbonizing said shapes and finally firmly co- 20 hering the carbonized product.
6. The method of making hard metal members comprising intimately intermixing finely divided powders of one or more refractory metals of the group consisting of tungsten, tantalum, titanium, 25 zirconium, chromium, thorium and rhenium, with finely divided powders of one or more base metals of the group consisting of iron, manganese, nickel, cobalt, silver and copper, sintering and alloying said mixture and then carbidizing the same, fine- 30 ly dividing the carbidized product and forming a plastic mass thereof, extruding said mass into a shape, carbonizing said shape and finally baking the carbonized product under reducing conditions.
- 35 7. The method of making hard metal members comprising intimately intermixing powders of a refractory metal with powders of a base metal, sintering and alloying said mixture and then carbidizing the same, finely dividing the carbidized 40 product and forming a plastic mass thereof, extruding said mass into a shape of the desired form, drying the same and cutting the dried shapes approximately to size, carbonizing said shapes and finally firmly cohering the carbonized 45 product.
8. The method of making hard metal members comprising intimately intermixing powders of a refractory metal with powders of a base metal, sintering, alloying and carbidizing the mixture, 50 comminuting the carbidized product, forming the same into a plastic mass, extruding said mass, drying the extruded shape, carbonizing the same and finally baking the product under reducing conditions.
- 55 9. The method of making hard metal members comprising intimately intermixing powders of a refractory metal with powders of a base metal, sintering, alloying and carbidizing the mixture, 60 comminuting the carbidized product, forming the same into a plastic mass, extruding said mass, drying the extruded shape, carbonizing the same and finally bonding together the carbide particles by heat.
- 65 10. The method of making hard metal members comprising intimately intermixing powders of a refractory metal with powders of a base metal, sintering, alloying and carbidizing the mixture, 65 comminuting the carbidized product, forming the same into a plastic mass, extruding said mass, drying the extruded shape, carbonizing the same and finally bonding together the carbide particles by heat.
- 70 11. The process of making hard metal members which includes the steps of forming a plastic mass of carbidized alloy particles and then extruding the said mass.
- 75 12. The process which comprises intimately intermixing refractory metal powders with base metal powders, alloying and carbidizing said mixture, comminuting said carbidized product, then mixing the same with a binder into a plastic mass, extruding the mass, drying the same, and then firmly uniting the mass by heating the same under reducing conditions.
- 80 13. The process of making hard metal members which comprises mixing, in finely divided form, one or more refractory metals adapted to form carbides and having melting points materially higher than 1500° C. with one or more metals also in finely divided state having melting points above 900° C., alloying said metals by heating 85 said mixture to a temperature of 700° C. to 900° C., carbidizing said alloyed metals, comminuting said carbides, plasticizing said comminuted product and then forming the desired member from said plastic material.
- 85 14. The process of making hard metal members which comprises mixing finely divided refractory metals of the group consisting of tungsten, tantalum, titanium, zirconium, chromium, thorium and rhenium with finely divided metals of the group consisting of iron, nickel, cobalt, manganese, silver and copper, alloying the finely divided metals in the mixture by heating the same to a temperature slightly below the melting point of the metal or metals of the said second group 90 in the mixture, carbidizing the metals thus alloyed, comminuting said carbides, plasticizing the comminuted product, and then forming the desired member from said plastic mixture.
- 95 15. The method of forming hard metal compositions which comprises intimately mixing and milling the finely divided metal powders, in dry state, of two or more refractory metals of the group consisting of tungsten, tantalum, titanium, zirconium, chromium, thorium, and rhenium, and one or more metals of the group consisting of iron, nickel, cobalt, manganese, silver and copper; then heating the mixture to a temperature below the melting point of the metal or metals of the second group and thereafter carbidizing the alloy 100 so formed.
16. The method of forming hard metal compositions which comprises intimately mixing and milling in dry state one or more refractory metal powders with one or more base metal powders, 105 alloying said metals by heating to a temperature below the melting point of the base metal or metals, and thereafter carbidizing the alloys so formed.